

## UNITED STATES PATENT OFFICE

2,063,351

HARDENING PHOTOGRAPHIC GELATIN  
EMULSIONS AND GELATIN SOLUTIONSCyril J. Staud and Richard M. Briggs, Rochester,  
N. Y., assignors, by mesne assignments, to  
Eastman Kodak Company, Jersey City, N. J., a  
corporation of New JerseyNo Drawing. Application August 4, 1934,  
Serial No. 738,559

16 Claims. (Cl. 95—7)

This invention relates to photographic materials and more particularly to the hardening of gelatin, either when applied as an emulsion layer on photographic films, plates, or papers, or when applied in the form of a solution as a simple coating or sizing for paper or similar materials.

In the preparation of photographic emulsions it has been the practice for many years to overcome the tendency of the gelatin to melt, or to swell during development, particularly at high temperatures, by addition of various so-called hardening agents, the most well-known of which appear to be chrome alum and formaldehyde. Other materials such as acrolein, glyoxal and derivatives of glyoxal have been proposed for this purpose, but none of these materials has proved to meet all the demands which have been put upon them, especially from the photographic standpoint.

We have now discovered, however, that the diketones are effective in enabling gelatin emulsions and gelatin layers in general to resist relatively elevated temperatures without undue swelling and, in the case of sensitized materials, to do so with less production of fog or desensitizing than other materials.

It is accordingly an object of the present invention to overcome the difficulties encountered in the use of known hardening agents and to provide a method whereby gelatin emulsions may be given a satisfactory degree of hardening. Another object is to provide a photographic emulsion which will resist relatively elevated temperatures without melting and which will do so without objectionable fogging or desensitizing. Another object is to provide a method of hardening gelatin solutions or layers in general whether in the form of photographic emulsions or merely in the form of a protective coating, applied to paper and similar surfaces. A further object is to provide gelatin layers which will be less subject to the phenomenon known as "after-hardening" in which the melting point of the gelatin rises considerably after storage, particularly storage in a moderately warm atmosphere. A still further object is to provide a gelatin solution or emulsion in which the newly discovered hardening agents of our invention may be used in conjunction with known hardening agents such as chrome alum and formaldehyde. Other objects will appear hereinafter.

We have found that the above objects may be accomplished by incorporating into the gelatin emulsion or solution one of the dialkyl, diaryl, or

alkaryl diketones, for example, diacetyl, acetyl caprolyl, acetyl benzoyl, or mixtures thereof.

In the following examples we have set forth several of the preferred embodiments of our invention, but they are included merely for purposes of illustration and not as a limitation thereof.

*Example I.*—To 200 c. c. of a moderately sensitive moderate gamma photographic emulsion comprising a silver halide there is added 0.2 gram of diacetyl after the emulsion has been melted and is being held at approximately 40° C. The diacetyl may be added as a 10 per cent solution in methanol or other suitable solvent in which case 2 c. c. of the solution are added. The emulsion is then coated on a plate or other support in the usual manner.

As illustrating the beneficial effects of the addition of a diketone to a gelatin in accordance with our invention, an emulsion produced as above can be satisfactorily processed at 100° F. employing developing bath, wash water, fixing bath and final wash at that temperature, whereas an ordinary gelatin emulsion not containing a hardener in accordance with our invention melts and runs off the plate at 85° F. The hardening appears somewhat progressive with time and is noticeably greater after, for instance, 14 days incubation at 113° F. Even under these conditions, diacetyl, for example, does not give rise to serious fog or desensitizing of the emulsion.

*Example II.*—To 200 c. c. of a gelatin emulsion of the same general type as that described in Example I there are added 2 c. c. of a 10% methanol solution of acetyl benzoyl the emulsion being melted and held at about 40° C. The emulsion is then coated on a suitable support and is found to process satisfactorily without objectionable softening or melting of the emulsion at temperatures as high as 85° F. It will be noted that the hardening effect is somewhat less drastic in this case, but this is due solely to the fact that a lower mol. per cent of the hardening agent is employed for the same amount of gelatin.

As is the case with the product obtained in Example I, the product showed an increase in melting point of only about 15° F. after incubation at 113° F. for 14 days.

*Example III.*—To 200 c. c. of a moderately sensitive photographic emulsion comprising a silver halide there is added 2 grams of acetyl caprolyl under the conditions of the previous examples and an emulsion is thereby produced which processes satisfactorily at 85° F. upon two

weeks incubation may be processed at temperatures as high as 100° F.

The above examples are, as indicated, merely illustrative and many changes may be made in the various manipulative procedures, temperatures, concentrations and ingredients within the scope of our invention depending on the type of gelatin used, and the results desired in the finished product. While we have chosen to illustrate our invention by specific reference to diacetyl, acetyl, caproyl and acetyl benzoyl the broad scope thereof includes the dialkyl ketones in general, of which diacetyl is possibly the most representative and including acetyl caproyl; the diaryl diketones, of which dibenzoyl is typical; and the alkaryl diketones such as acetyl benzoyl.

Our invention is applicable not only to the manufacture of photographic emulsions of satisfactory hardening properties, but may likewise be applied to the manufacture of gelatin solutions which are used for producing other types of coatings or layers on paper, cloth, film and other surfaces.

We have also found as indicated above that the hardening effect of these diketones increases with increasing pH to an optimum value, which may vary with different gelatines, but in these used was found to be of the order of pH=8, and that they may be used as an adjunct to other hardening agents, such as various aliphatic and other aldehydes, including formaldehyde and also chrome alum.

What we claim is:

1. In the manufacture of photographic articles provided with a hardened gelatin layer, the step which comprises hardening the gelatin by causing it to react with a diketone, whereby a condensation product of gelatin and the diketone is formed.

2. In the manufacture of photographic articles provided with a hardened gelatin layer, the step which comprises hardening the gelatin by causing it to react with a diketone selected from the group comprising the dialkyl diketones, the diaryl diketones, and the alkaryl diketones, whereby a condensation product of gelatin and the diketone is formed.

3. In the manufacture of photographic articles provided with a hardened gelatin layer, the step which comprises hardening the gelatin by causing it to react with diacetyl, whereby a condensation product of gelatin and diacetyl is formed.

4. In the manufacture of photographic articles provided with a hardened gelatin layer, the step which comprises hardening the gelatin by causing it to react with acetyl caproyl, whereby a condensation product of gelatin and acetyl caproyl is formed.

5. In the manufacture of photographic articles provided with a hardened gelatin layer, the step which comprises hardening the gelatin by caus-

ing it to react with acetyl benzoyl, whereby a condensation product of gelatin and acetyl benzoyl is formed.

6. An article of manufacture comprising a sheet material having thereon a layer of gelatin, said layer containing the condensation product of gelatin and a diketone.

7. A photographic material provided with a gelatin silver halide emulsion layer, said layer containing the condensation product of gelatin and a diketone.

8. A photographic material provided with a gelatin silver halide emulsion layer, said layer containing the condensation product of gelatin and a diketone selected from the group comprising the dialkyl diketones, the diaryl diketones, and the alkaryl diketones.

9. A photographic material provided with a gelatin silver halide emulsion layer, said layer containing the condensation product of gelatin and diacetyl.

10. A photographic material provided with a gelatin silver halide emulsion layer, said layer containing the condensation product of gelatin and acetyl caproyl.

11. A photographic material provided with a gelatin silver halide emulsion layer, said layer containing the condensation product of gelatin and acetyl benzoyl.

12. A composition of matter comprising a solution of gelatin containing diacetyl, said solution being adapted for the production of a hardened gelatin layer containing the condensation product of gelatin and diacetyl.

13. In the manufacture of photographic articles provided with a hardened gelatin layer, the step which comprises hardening the gelatin by causing it to react with a diketone in which the carbonyl groups are adjacent, whereby a condensation product of gelatin and the diketone is formed.

14. The process of producing a hardened gelatin emulsion layer which comprises adding a solution of a diketone to the melted emulsion at a temperature of approximately 40° C., whereby a condensation product of gelatin and the diketone is formed, and thereafter coating the melted emulsion on a suitable support.

15. A composition of matter comprising a solution of gelatin containing acetyl caproyl and adapted for the production of a hardened gelatin layer containing the condensation product of gelatin and acetyl caproyl.

16. A composition of matter comprising a solution of gelatin containing acetyl benzoyl and adapted for the production of a hardened gelatin layer containing the condensation product of gelatin and acetyl benzoyl.

CYRIL J. STAUD.

RICHARD M. BRIGGS.